

Patented Sept. 5, 1922.

1,428,170

## UNITED STATES PATENT OFFICE.

FREDERICK LAIST, FREDERICK F. FRICK, ERNEST KLEPETKO, AND LYNDALL P. DAVIDSON, OF ANACONDA, MONTANA, ASSIGNORS TO ANACONDA COPPER MINING COMPANY, OF ANACONDA, MONTANA, A CORPORATION OF MONTANA.

### PROCESS FOR COLORING METALLIC COPPER.

No Drawing.

Application filed November 29, 1921. Serial No. 518,647.

To all whom it may concern:

Be it known that we, FREDERICK LAIST, FREDERICK F. FRICK, ERNEST KLEPETKO, and LYNDALL P. DAVIDSON, citizens of the United States, residing at Anaconda, in the county of Deer Lodge and State of Montana, have invented certain new and useful Improvements in Processes for Coloring Metallic Copper, of which the following is a specification.

This invention relates to the coloring of metallic copper by wet chemical processes.

It is the object of this invention to provide a process by which metallic copper used for structural or decorative purposes may be quickly and economically given certain desirable hues or colors of the order obtainable only after an exposure of many years to atmospheric conditions.

It is another object to provide a process by which a relatively wide range and diversity of colors may be obtained.

The process may be carried out as follows:

The object to be treated, for instance copper sheets for roofing, are first carefully pickled in hot dilute sulphuric acid. After washing they are suspended in an aqueous preferably saturated solution of copper nitrate and copper chloride. The time of immersion depends on the temperature of the bath. Fifteen minutes at 90° to 100° C. and twelve hours at room temperature give equally good results. The bath of copper nitrate and chloride must contain no free acid. It usually contains basic copper salts in suspension.

After immersion under conditions as above mentioned the sheets, on removal, are covered with a blue coating, a basic copper salt.

The sheet is washed with water and an excess or loose coating is rubbed off.

After washing the sheets are immersed in a dilute caustic soda solution for approximately ten minutes, after which they are washed with water. The color is deepened and densified by the caustic soda treatment. The color varies from blue to a greenish blue depending upon the proportions of copper nitrate and copper chloride in the bath. In general the greenish hue increases with an increased proportion of copper chloride.

The sheets are then washed after the caustic soda treatment.

In order to obtain a wider range of colors, the sheets after the caustic soda treatment may be immersed in a dilute ferrous sulphate solution. Depending upon the time of immersion, a range from malachite green through olive green to reddish brown may be obtained.

After the ferrous sulphate treatment the sheets are again washed.

When the desired hue has been obtained, the coating is made permanent by immersion in a dilute solution of sodium silicate, followed by washing.

The coloring bath may be kept in condition for carrying out the process by addition of copper nitrate, copper chloride and nitric acid. Excess basic salts are dissolved by the nitric acid.

In the foregoing we have described what we consider the best manner of carrying out the invention. It should be understood, however, that the process may be modified in various respects within the scope of the invention.

The first three steps described serve the purpose of producing colored deposit, while the last step has the object to render the deposit insoluble.

The treatment with a mixture of copper nitrate and copper chloride, followed by treatment with caustic soda produces a brilliant bluish-green which for certain purposes may be the ultimate color effect desired.

The action of a copper nitrate solution alone when followed by a caustic soda treatment produces a color of the order of azurite blue. For certain purposes also this color may correspond to the final effect desired.

However for most practical purposes these colors are too pronounced and conspicuous and must be more or less modified by the application of a ferrous sulphate solution. It should be noted that while we prefer ferrous sulphate, which acts as a reducing agent, other reducing agents may be used, as for instance sodium oxalate or sodium sulphite which convert the bluish-green color produced by the first two steps described above in detail to a yellow-green.

While we consider sodium hydroxide as

the most desirable alkali for the purposes above described, other alkaline solutions may be used with satisfactory results, as for instance a mixture of sodium carbonate and 5 sodium hydroxide.

It is thus apparent that, within a certain range previously pointed out, it is easily possible to control the formation of colored 10 deposits and produce a substantially uniform final color effect of predetermined hue.

The use of sodium silicate for the purpose of making the colored deposit insoluble has the commercial advantage of being a very 15 cheap reagent. So far as the desired physical result of it is concerned, other substances, for instance sodium sulphite, might be used instead.

The process described with the various 20 modifications of which it is susceptible has been developed primarily for the purpose of producing an artificial copper "rust" on copper shingles so as to give a copper roof initially a more pleasing predetermined permanent color effect. As above suggested, 25 however, the process is equally applicable to the coloring of other copper or cupriferous objects, for instance brass or bronze candlesticks, ash trays, and objects or art in general where it is desired to "antique" the object, as well as brass shingles for a cheaper 30 metal roofing material.

We claim:

1. In a process of producing a colored 35 coating on cupriferous bodies including copper, the step which consists in subjecting a body to the action of a substantially concentrated aqueous solution of a copper salt.

2. In a process of producing a colored 40 coating on cupriferous bodies including copper, the step which consists in subjecting a body to the action of a substantially concentrated aqueous solution of copper nitrate.

3. In a process of producing a colored 45 coating on cupriferous bodies including copper, the step which consists in subjecting a body to the action of a substantially concentrated aqueous solution of copper nitrate and copper chloride.

4. In a process of producing a colored 50 coating upon bodies of metallic copper, the step which consists in subjecting a body to the action of a substantially concentrated aqueous solution of copper nitrate and copper chloride.

5. In a process of producing a colored 55 coating on cupriferous bodies including copper, the steps which consist in subjecting a body to the action of a substantially concentrated aqueous solution of a copper 60 salt reacting with the body to produce thereon a basic copper salt deposit and then subjecting the body to the action of an aqueous solution of an alkaline reagent.

6. In a process of producing a colored 65 coating on cupriferous bodies including cop-

per, the steps which consist in subjecting a body to the action of a substantially concentrated aqueous solution of copper nitrate and thereafter subjecting the body to the action of an aqueous solution of an alkaline 70 reagent.

7. In a process of producing a colored 75 coating on cupriferous bodies including copper, the steps which consist in subjecting a body to the action of a substantially concentrated aqueous solution of copper nitrate and copper chloride and thereafter subjecting the body to the action of an aqueous solution of an alkaline reagent.

8. In a process of producing a colored 80 coating on cupriferous bodies including copper, the steps which consist in subjecting a body to the action of a substantially concentrated aqueous solution of a copper salt reacting with the body to produce thereon 85 a basic copper salt deposit and then subjecting the body to the action of an aqueous solution of sodium hydroxide.

9. In a process of producing a colored 90 coating on cupriferous bodies including copper, the steps which consist in subjecting a body to the action of a substantially concentrated aqueous solution of copper nitrate and thereafter subjecting the body to the action of an aqueous solution of sodium 95 hydroxide.

10. In a process of producing a colored coating on cupriferous bodies including copper, the steps which consist in subjecting a body to the action of an aqueous solution 100 of copper nitrate and copper chloride and thereafter subjecting the body to the action of an aqueous solution of sodium hydroxide.

11. In a process of producing a colored 105 coating on bodies of metallic copper, the steps which consist in subjecting a body to the action of a substantially concentrated aqueous solution of copper nitrate and copper chloride and thereafter subjecting the body to the action of an alkaline reagent.

12. In a process of producing a colored 110 coating on cupriferous bodies including copper, the steps which consist in subjecting a body to the action of an aqueous solution of a copper salt reacting with the body to produce thereon a basic copper salt deposit and thereafter subjecting the body to the action of an aqueous solution of a reducing agent.

13. In a process of producing a colored 115 coating on cupriferous bodies including copper, the steps which consist in subjecting a body to the action of an aqueous solution of a copper salt reacting with the body to produce thereon a basic copper salt deposit and thereafter subjecting the body to the action of an aqueous solution of a ferrous salt.

14. In a process of producing a colored 120 coating on cupriferous bodies including copper, the steps which consist in subjecting a body to the action of an aqueous solution of a ferrous salt.

a body to the action of an aqueous solution of a copper salt reacting with the body to produce thereon a basic copper salt deposit and thereafter subjecting the body to the action of an aqueous solution of ferrous sulphate.

15. In a process of producing a colored coating on cupriferous bodies including copper, the steps which consist in subjecting a body to the action of an aqueous solution of a copper salt reacting with the body to produce thereon a basic copper salt deposit, then subjecting the body to the action of an aqueous solution of an alkaline reagent and then subjecting the body to the action of an aqueous solution of a reducing agent.

16. Process according to claim 13 in which the copper salt solution contains copper nitrate.

20 17. Process according to claim 13 in which the copper salt solution contains copper nitrate and copper chloride.

18. Process according to claim 13 in which the reducing agent is ferrous sulphate.

25 19. In a process of producing a colored coating on cupriferous bodies including copper, the steps which consist in subjecting the body to the action of aqueous solution of a copper salt reacting with the body to produce thereon a basic copper salt deposit and thereafter subjecting the body to the action of an aqueous solution of a salt reacting with the deposit formed to make it insoluble in water.

30 20. Process according to claim 17 in which the last mentioned salt is sodium silicate.

21. In a process of producing a colored coating on cupriferous bodies including copper, the steps which consist in subjecting the body to the action of aqueous solution of a copper salt reacting with the body to pro-

duce thereon a basic copper salt deposit, then subjecting the body to the action of an aqueous solution of an alkaline reagent and thereafter subjecting the body to the action of a salt reacting upon the salt deposit to make it insoluble in water.

22. In a process of producing a colored coating on cupriferous bodies including copper, the steps which consist in subjecting the body to the action of aqueous solution of a copper salt reacting with the body to produce thereon a basic copper salt deposit, thereafter subjecting the body to the action of an aqueous solution of a reducing agent and then subjecting the body to the action of an aqueous solution of a salt reacting upon the salt deposit to make it insoluble in water.

23. A process of producing a colored coating on cupriferous bodies including copper, which consists in immersing a body in an aqueous solution containing copper nitrate, then in an aqueous solution of sodium hydroxide, then in an aqueous solution of ferrous sulphate and then in an aqueous solution of sodium silicate.

24. A process of producing a colored coating on cupriferous bodies including copper, which consists in immersing a body in an aqueous solution containing copper nitrate and copper chloride, then in an aqueous solution of sodium hydroxide, then in an aqueous solution of ferrous sulphate and then in an aqueous solution of sodium silicate.

In testimony whereof, we affix our signatures.

FREDERICK LAIST.  
FREDERICK F. FRICK.  
ERNEST KLEPETKO.  
LYNDALL P. DAVIDSON.